



US010589344B2

(12) **United States Patent**  
**Bewlay et al.**

(10) **Patent No.:** **US 10,589,344 B2**  
(45) **Date of Patent:** **\*Mar. 17, 2020**

(54) **MOLD COMPOSITIONS AND METHODS FOR CASTING TITANIUM AND TITANIUM ALUMINIDE ALLOYS**

(71) Applicant: **GENERAL ELECTRIC COMPANY**, Schenectady, NY (US)

(72) Inventors: **Bernard Patrick Bewlay**, Niskayuna, NY (US); **Stephen Bancheri**, Albany, NY (US); **Michael Weimer**, Loveland, OH (US); **Joan McKiever**, Rock Mount, VA (US); **Brian Ellis**, Mayfield, NY (US)

(73) Assignee: **General Electric Company**, Schenectady, NY (US)

(\*) Notice: Subject to any disclaimer, the term of this patent is extended or adjusted under 35 U.S.C. 154(b) by 140 days.

This patent is subject to a terminal disclaimer.

(21) Appl. No.: **15/724,472**

(22) Filed: **Oct. 4, 2017**

(65) **Prior Publication Data**

US 2018/0029107 A1 Feb. 1, 2018

**Related U.S. Application Data**

(60) Continuation of application No. 14/595,533, filed on Jan. 13, 2015, now Pat. No. 9,802,243, which is a (Continued)

(51) **Int. Cl.**  
**B22C 1/00** (2006.01)  
**B22C 9/22** (2006.01)

(Continued)

(52) **U.S. CL.**  
CPC ..... **B22C 1/00** (2013.01); **B22C 9/04** (2013.01); **B22C 9/22** (2013.01); **B22D 21/022** (2013.01); **B22C 7/02** (2013.01)

(58) **Field of Classification Search**  
CPC .... B22C 1/00; B22C 7/02; B22C 9/04; B22C 9/22; B22D 21/02; B22D 21/022  
(Continued)

(56) **References Cited**

U.S. PATENT DOCUMENTS

3,955,616 A 5/1976 Gigliotti, Jr. et al.  
8,708,033 B2 4/2014 Bewlay et al.  
(Continued)

FOREIGN PATENT DOCUMENTS

JP H08-281371 A 10/1996

OTHER PUBLICATIONS

Barbosa, J. et al., "Influence of superheating on casting of  $\gamma$ -TiAl", *Intermetallics*, vol. 15, No. 7, pp. 945-955, (Jul. 2007).  
(Continued)

*Primary Examiner* — Kevin P Kerns

(74) *Attorney, Agent, or Firm* — Armstrong Teasdale LLP

(57) **ABSTRACT**

A method for forming a mold for casting a titanium-containing article, the method including combining calcium aluminate with a liquid to produce an initial slurry of calcium aluminate and adding oxide particles into the initial slurry to create a final slurry. The method further includes introducing the final slurry into a mold cavity that contains a fugitive pattern and allowing the final slurry to cure in the mold cavity to form a mold of a titanium-containing article.

**19 Claims, 6 Drawing Sheets**



**Related U.S. Application Data**

division of application No. 13/407,917, filed on Feb. 29, 2012, now Pat. No. 8,932,518.

**(51) Int. Cl.**

*B22C 9/04* (2006.01)  
*B22D 21/02* (2006.01)  
*B22C 7/02* (2006.01)

**(58) Field of Classification Search**

USPC ..... 164/519, 520, 529  
See application file for complete search history.

**(56) References Cited****U.S. PATENT DOCUMENTS**

|                 |         |               |                 |
|-----------------|---------|---------------|-----------------|
| 8,906,292 B2    | 12/2014 | Bewlay et al. |                 |
| 8,932,518 B2 *  | 1/2015  | Bewlay et al. | ..... B22C 9/04 |
|                 |         |               | 420/417         |
| 8,992,824 B2    | 3/2015  | Bewlay et al. |                 |
| 9,511,417 B2    | 12/2016 | Bewlay et al. |                 |
| 9,592,548 B2    | 3/2017  | Bewlay et al. |                 |
| 9,721,044 B2    | 8/2017  | Bewlay et al. |                 |
| 9,802,243 B2 *  | 10/2017 | Bewlay et al. | ..... B22C 9/04 |
| 2013/0108459 A1 | 5/2013  | Bewlay et al. |                 |

**OTHER PUBLICATIONS**

Gomes, F. et al., "Induction melting of  $\gamma$ -TiAl in CaO crucibles," *Intermetallics*, vol. 16, No. 11, pp. 1292-1297, (Nov. 2008).

Kuang, J.P. et al., "Investigation into refractories as crucible and mould materials for melting and casting  $\gamma$ -TiAl alloys," *Materials Science and Technology*, vol. 16, Issue 9, pp. 1007-1016, (Sep. 2000).

Kuang, J.P. et al., "A study of refractories as crucible and mould materials for melting and casting  $\gamma$ -TiAl alloys," *International Journal of Cast Metals Research*, vol. 13, Issue 2001, pp. 277-292 (2001).

Menand, A. et al., "Interstitial solubility in  $\gamma$  and  $\alpha_2$  phases of TiAl-based alloys," *Acta Materialia*, vol. 44, No. 12, pp. 4729-4737, (Dec. 1996) (Abstract).

Machine translation and Notification of Reasons for Refusal issued in connection with corresponding JP Application No. 2013-031615 dated Jan. 10, 2017.

Machine translation and Decision to Grant issued in connection with corresponding JP Application No. 2013-031615 dated Apr. 18, 2017.

\* cited by examiner

**FIG. 1a****FIG. 1b**

FIG. 2a



FIG. 2b



FIG. 3



2 microns

FIG. 4

10 microns

700

COMBINING CALCIUM ALUMINATE WITH A LIQUID TO PRODUCE A SLURRY OF CALCIUM ALUMINATE IN THE LIQUID

-705

ADDING OXIDE PARTICLES INTO THE SLURRY

-707

INTRODUCING THE SLURRY INTO A MOLD CAVITY THAT CONTAINS A FUGITIVE PATTERN

-710

ALLOWING THE SLURRY TO CURE IN THE MOLD CAVITY TO FORM A MOLD OF A TITANIUM-CONTAINING ARTICLE

-715

**FIG. 5a**

OBTAINING AN INVESTMENT CASTING MOLD COMPOSITION COMPRISING CALCIUM ALUMINATE AND ALUMINUM OXIDE

-725

POURING SAID INVESTMENT CASTING MOLD COMPOSITION INTO A VESSEL CONTAINING A FUGITIVE PATTERN

-730

CURING SAID INVESTMENT CASTING MOLD COMPOSITION

-735

REMOVING SAID FUGITIVE PATTERN FROM THE MOLD

-740

FIRING THE MOLD

-745

PREHEATING THE MOLD TO A MOLD CASTING TEMPERATURE

-750

POURING MOLTEN TITANIUM OR TITANIUM ALLOY INTO THE HEATED MOLD

-755

SOLIDIFYING THE MOLTEN TITANIUM OR TITANIUM ALLOY AND FORMING A SOLIDIFIED TITANIUM OR TITANIUM ALLOY CASTING

-760

REMOVING THE SOLIDIFIED TITANIUM ALLOY CASTING FROM THE MOLD

**FIG. 5b**



FIG. 6



FIG. 7

## 1

**MOLD COMPOSITIONS AND METHODS  
FOR CASTING TITANIUM AND TITANIUM  
ALUMINIDE ALLOYS**

**CROSS-REFERENCE TO RELATED  
APPLICATION**

This application is a continuation of U.S. application Ser. No. 14/595,533, filed on Jan. 13, 2015 and entitled Methods for Casting Titanium and Titanium Aluminide Alloys, and patented as U.S. Pat. No. 9,802,243, on Oct. 31, 2017, which is a divisional of U.S. application Ser. No. 13/407,917, filed on Feb. 29, 2012 and entitled Mold and Facecoat Compositions, and patented as U.S. Pat. No. 8,932,518 on Jan. 13, 2015, which are both hereby expressly incorporated herein by reference in their entirety.

**BACKGROUND**

Modern gas or combustion turbines must satisfy the highest demands with respect to reliability, weight, power, economy, and operating service life. In the development of such turbines, the material selection, the search for new suitable materials, as well as the search for new production methods, among other things, play an important role in meeting standards and satisfying the demand.

The materials used for gas turbines may include titanium alloys, nickel alloys (also called super alloys) and high strength steels. For aircraft engines, titanium alloys are generally used for compressor parts, nickel alloys are suitable for the hot parts of the aircraft engine, and the high strength steels are used, for example, for compressor housings and turbine housings. The highly loaded or stressed gas turbine components, such as components for a compressor for example, are typically forged parts. Components for a turbine, on the other hand, are typically embodied as investment cast parts.

Although investment casting is not a new process, the investment casting market continues to grow as the demand for more intricate and complicated parts increase. Because of the great demand for high quality, precision castings, there continuously remains a need to develop new ways to make investment castings more quickly, efficiently, cheaply and of higher quality.

Conventional investment mold compounds that consist of fused silica, cristobalite, gypsum, or the like, that are used in casting jewelry and dental prostheses industries are generally not suitable for casting reactive alloys, such as titanium alloys. One reason is because there is a reaction between mold titanium and the investment mold.

There is a need for a simple investment mold that does not react significantly with titanium and titanium aluminide alloys. Approaches have been adopted previously with ceramic shell molds for titanium alloy castings. In the prior examples, in order to reduce the limitations of the conventional investment mold compounds, several additional mold materials have been developed. For example, an investment compound was developed of an oxidation-expansion type in which magnesium oxide or zirconia was used as a main component and metallic zirconium was added to the main constituent to compensate for the shrinkage due to solidification of the cast metal. There is thus also a need for simple and reliable investment casting methods which allow easy extraction of near-net-shape metal or metal alloys from an investment mold that does not react significantly with the metal or metal alloy.

## 2

**SUMMARY**

Aspects of the present disclosure provide casting mold compositions, methods of casting, and cast articles that overcome the limitations of the conventional techniques. Though some aspect of the disclosure may be directed toward the fabrication of components for the aerospace industry, for example, engine turbine blades, aspects of the present disclosure may be employed in the fabrication of any component in any industry, in particular, those components containing titanium and/or titanium alloys.

One aspect of the present disclosure is a mold for casting a titanium-containing article, comprising: a calcium aluminate cement comprising calcium monoaluminate, calcium dialuminate, and mayenite, wherein the mold has an intrinsic facecoat of about 10 microns to about 250 microns between the bulk of the mold and the mold cavity. In one embodiment, the facecoat is a continuous intrinsic facecoat. In one embodiment, the mold as recited further comprises silica, for example, colloidal silica.

The mold, in one example, comprises the bulk of the mold and an intrinsic facecoat, with the bulk of the mold and the intrinsic facecoat having different compositions, and the intrinsic facecoat comprising calcium aluminate with a particle size of less than about 50 microns. In another embodiment, the mold comprises the bulk of the mold and an intrinsic facecoat, wherein the bulk of the mold and the intrinsic facecoat have different compositions and wherein the bulk of the mold comprises alumina particles larger than about 50 microns. The mold, in another example, comprises the bulk of the mold and an intrinsic facecoat, wherein the bulk of the mold comprises alumina particles larger than about 50 microns and the intrinsic facecoat comprises calcium aluminate particles less than about 50 microns in size.

In certain embodiments, the intrinsic facecoat has, by weight fraction, at least 20 percent more calcium monoaluminate than does the bulk of the mold. In one embodiment, the intrinsic facecoat has, by weight fraction, at least 20 percent less alumina than does the bulk of the mold. In another embodiment, the intrinsic facecoat has, by weight fraction, at least 20 percent more calcium aluminate, at least 20 percent less alumina, and at least 50 percent less mayenite than does the bulk of the mold.

The weight fraction of calcium monoaluminate in the intrinsic facecoat is, in one example, more than 0.60 and the weight fraction of mayenite is less than 0.10. In one embodiment, the calcium monoaluminate in the bulk of the mold comprises a weight fraction of about 0.05 to 0.95, and the calcium monoaluminate in the intrinsic facecoat is about 0.10 to 0.90. In another embodiment, the calcium dialuminate in the bulk of the mold comprises a weight fraction of about 0.05 to about 0.80, and the calcium dialuminate in the intrinsic facecoat is about 0.05 to 0.90. In yet another embodiment, the mayenite in the bulk of the mold composition comprises a weight fraction of about 0.01 to about 0.30, and the mayenite in the intrinsic facecoat is about 0.001 to 0.05. In a particular embodiment, the calcium monoaluminate in the bulk of the mold comprises a weight fraction of about 0.05 to 0.95, and the calcium monoaluminate in the intrinsic facecoat is about 0.1 to 0.90; the calcium dialuminate in the bulk of the mold comprises a weight fraction of about 0.05 to about 0.80, and the calcium dialuminate in the intrinsic facecoat is about 0.05 to 0.90; and wherein the mayenite in the bulk of the mold composition comprises a weight fraction of about 0.01 to about 0.30, and the mayenite in the intrinsic facecoat is about 0.001 to 0.05.

In one example, the mold further comprises aluminum oxide particles in the bulk of the mold that are less than about 500 microns in outside dimension. In one example, the aluminum oxide particles comprise from about 40% by weight to about 68% by weight of the composition used to make the mold. These aluminum oxide particles may be hollow. In another embodiment, the calcium aluminate cement comprises more than 30% by weight of the composition used to make the mold. In one embodiment, the mold further comprises more than about 10% by weight and less than about 50% by weight of the mold composition in calcium oxide.

In one example, the mold further comprises aluminum oxide particles, magnesium oxide particles, calcium oxide particles, zirconium oxide particles, titanium oxide particles, silicon oxide particles, or compositions thereof.

The percentage of solids in an initial calcium aluminate—liquid cement mixture used to make the mold is, in one example, from about 71 to about 78%. In another example, the percentage of solids in the final calcium aluminate—liquid cement mixture with the large scale alumina, used to make the mold, is from about 75% to about 90%.

One aspect of the present disclosure is a titanium-containing article formed in the mold recited in claim 1. The article, in one example, comprises a titanium aluminide-containing turbine blade. In one aspect, the present disclosure is the mold as recited herein, wherein the mold forms a titanium-containing article. In one related embodiment, the titanium-containing article comprises a titanium aluminide-containing turbine blade.

One aspect of the present disclosure is a facecoat composition of a mold that is used for casting a titanium-containing article, the facecoat composition comprising: calcium monoaluminate, calcium dialuminate, and mayenite, wherein the facecoat composition is an intrinsic facecoat, is about 10 microns to about 250 microns thick, and is located between the bulk of the mold and the surface of the mold that opens to the mold cavity. The facecoat comprises, in one example, of calcium aluminate with a particle size of less than about 50 microns. In one embodiment, the facecoat composition further comprises silica, for example, colloidal silica.

In one embodiment, the intrinsic facecoat has, by weight fraction, at least 20 percent more calcium aluminate, at least 20 percent less alumina, and at least 50 percent less mayenite than does the bulk of the mold. The weight fraction of calcium monoaluminate in the intrinsic facecoat is, in one example, more than 0.60 and the weight fraction of mayenite is less than 0.10. In one embodiment, the calcium monoaluminate in the intrinsic facecoat comprises a weight fraction of 0.10 to 0.90; the calcium dialuminate in the intrinsic facecoat comprises a weight fraction of 0.05 to 0.90; and the mayenite in the intrinsic facecoat comprises a weight fraction of 0.001 to 0.05.

One aspect of the present disclosure is a method for forming a casting mold for casting a titanium-containing article, the method comprising: combining calcium aluminate with a liquid to produce a slurry of calcium aluminate, wherein the percentage of solids in the initial calcium aluminate/liquid mixture is about 70% to about 80% and the viscosity of the slurry is about 10 to about 250 centipoise; adding oxide particles into the slurry such that the solids in the final calcium aluminate/liquid mixture with the large-scale (greater than 50 microns) oxide particles is about 75% to about 90%; introducing the slurry into a mold cavity that

contains a fugitive pattern; and allowing the slurry to cure in the mold cavity to form a mold of a titanium-containing article.

One aspect of the present disclosure is a casting method for titanium and titanium alloys comprising: obtaining an investment casting mold composition comprising calcium aluminate and aluminum oxide, wherein the calcium aluminate is combined with a liquid to produce a slurry of calcium aluminate, and wherein the solids in the final calcium aluminate/liquid mixture with the large scale alumina is about 75% to about 90%, and wherein the resulting mold has an intrinsic facecoat; pouring the investment casting mold composition into a vessel containing a fugitive pattern; curing the investment casting mold composition; removing the fugitive pattern from the mold; firing the mold; preheating the mold to a mold casting temperature; pouring molten titanium or titanium alloy into the heated mold; solidifying the molten titanium or titanium alloy and forming a solidified titanium or titanium alloy casting; and removing the solidified titanium or titanium alloy casting from the mold. In one embodiment, a titanium or titanium alloy article is claimed that is made by the casting method as taught herein.

One aspect of the present disclosure is a mold composition for casting a titanium-containing article, comprising: a calcium aluminate cement comprising calcium monoaluminate, calcium dialuminate, and mayenite. In one embodiment, the mold composition further comprises hollow particles of aluminum oxide. Another aspect of the present disclosure is a titanium-containing article casting-mold composition comprising calcium aluminate. For instance, an aspect of the present disclosure may be uniquely suited to providing mold compositions to be used in molds for casting titanium-containing and/or titanium alloy-containing articles or components, for example, titanium containing turbine blades.

These and other aspects, features, and advantages of this disclosure will become apparent from the following detailed description of the various aspects of the disclosure taken in conjunction with the accompanying drawings.

#### BRIEF DESCRIPTION OF THE FIGURES

The subject matter, which is regarded as the invention, is particularly pointed out and distinctly claimed in the claims at the conclusion of the specification. The foregoing and other features and advantages of the disclosure will be readily understood from the following detailed description of aspects of the invention taken in conjunction with the accompanying drawings in which:

FIGS. 1a and 1b show one example of the mold microstructure after high temperature firing with the backscattered electron imaging scanning electron microscope images of the cross section of the mold fired at 1000 degrees Celsius, wherein FIG. 1a points to the alumina particles present and FIG. 1b points to the calcium aluminate cement. FIG. 1a also shows the mold microstructure, showing the bulk of the mold, the location of the intrinsic facecoat, and the internal surface of the mold/mold cavity.

FIG. 2a and FIG. 2b show one example of the mold microstructure after high temperature firing with the backscattered electron imaging scanning electron microscope images of the cross section of the mold fired at 1000 degrees Celsius, wherein FIG. 2a points to calcium aluminate cement and fine-scale alumina particles present and FIG. 2b points to an alumina particle. FIG. 2b also shows the mold

microstructure, showing the bulk of the mold, the location of the intrinsic facecoat, and the internal surface of the mold/mold cavity.

FIGS. 3 and 4 show examples of the mold microstructure after high temperature firing, showing alumina and calcium monoaluminate, wherein the calcium monoaluminate reacts with alumina to form calcium dialuminate, and wherein the mold in one example is fired to minimize mayenite content.

FIG. 5a shows a flow chart, in accordance with aspects of the disclosure, illustrating a method for forming a casting mold for casting a titanium-containing article.

FIG. 5b shows a flow chart, in accordance with aspects of the disclosure, illustrating a casting method for titanium and titanium alloys.

FIG. 6 shows the thermal conductivity of the bulk of the mold as a function of temperature; the thermal conductivity of the mold is compared with the thermal conductivity of monolithic alumina (NIST data).

FIG. 7 shows a schematic of the mold with the facecoat. FIG. 7a shows the mold with the intrinsic facecoat that is, for example, approximately 100 microns thick. The schematic shows the intrinsic facecoat with the mold cavity and calcium aluminate mold positions also indicated. FIG. 7b shows the mold with the extrinsic facecoat that is approximately 100 microns thick. The schematic shows the extrinsic facecoat with the mold cavity and calcium aluminate mold positions also indicated.

#### DETAILED DESCRIPTION

The present disclosure relates generally to mold compositions and methods of mold making and articles cast from the molds, and, more specifically, to mold compositions and methods for casting titanium-containing articles, and titanium-containing articles so molded.

The manufacture of titanium based components by investment casting of titanium and its alloys in investment shell molds poses problems from the standpoint that the castings should be cast to “near-net-shape.” That is, the components may be cast to substantially the final desired dimensions of the component, and require little or no final treatment or machining. For example, some conventional castings may require only a chemical milling operation to remove any alpha case present on the casting. However, any sub-surface ceramic inclusions located below the alpha case in the casting are typically not removed by the chemical milling operation and may be formed due to the reaction between the mold facecoat and any reactive metal in the mold, for example, reactive titanium aluminide.

The present disclosure provides a new approach for casting near-net-shape titanium and titanium aluminide components, such as, turbine blades or airfoils. Embodiments of the present disclosure provide compositions of matter for investment casting molds and casting methods that provide improved titanium and titanium alloy components for example, for use in the aerospace, industrial and marine industry. In some aspects, the mold composition provides a mold that contain phases that provide improved mold strength during mold making and/or increased resistance to reaction with the casting metal during casting. The molds according to aspects of the disclosure may be capable of casting at high pressure, which is desirable for near-net-shape casting methods. Mold compositions, for example, containing calcium aluminate cement and alumina particles, and preferred constituent phases, have been identified that provide castings with improved properties.

In one aspect, the constituent phases of the mold comprise calcium monoaluminate ( $\text{CaAl}_2\text{O}_4$ ). The present inventors found calcium monoaluminate desirable for at least two reasons. First, it is understood by the inventors that calcium monoaluminate promotes hydraulic bond formation between the cement particles during the initial stages of mold making, and this hydraulic bonding is believed to provide mold strength during mold construction. Second, it is understood by the inventors that calcium monoaluminate experiences a very low rate of reaction with titanium and titanium aluminide based alloys. In a certain embodiment, calcium monoaluminate is provided to the mold composition of the present disclosure, for example, the investment molds, in the form of calcium aluminate cement. In one aspect, the mold composition comprises a mixture of calcium aluminate cement and alumina, that is, aluminum oxide.

In one aspect of the disclosure, the mold composition provides minimum reaction with the alloy during casting, and the mold provides castings with the required component properties. External properties of the casting include features such as shape, geometry, and surface finish. Internal properties of the casting include mechanical properties, microstructure, defects (such as pores and inclusions) below a specified size and within allowable limits.

In one embodiment, the mold contains a continuous intrinsic facecoat between the bulk of the mold and the mold cavity. In a related embodiment, the intrinsic facecoat is about 50 microns to about 250 microns. In certain instances, the facecoat comprises of calcium aluminate with a particle size of less than about 50 microns. The mold composition may be such that the bulk of the mold comprises alumina and particles larger than about 50 microns. In a certain embodiment, the facecoat has less alumina than the bulk of the mold, and wherein the facecoat has more calcium aluminate than the bulk of the mold.

The percentage of solids in the initial calcium aluminate—liquid cement mix, and the solids in the final calcium aluminate—liquid cement mix are a feature of the present disclosure. In one example, the percentage of solids in the initial calcium aluminate—liquid cement mix is from about 71% to about 78%. In one example, the percentage of solids in the initial calcium aluminate—liquid cement mix is from about 70% to about 80%. In another example, the solids in the final calcium aluminate—liquid cement mix with the large scale alumina (>100 microns) alumina particles is from about 75% to about 90%. The initial calcium aluminate cement and the fine-scale (less than 10 micron) alumina are mixed with water to provide a uniform and homogeneous slurry; the final mold mix is formed by adding large-scale (greater than 100 microns) alumina to the initial slurry and mixing for between 2 and 15 minutes to achieve a uniform mix.

The mold composition of one aspect of the present disclosure provides for low-cost casting of titanium aluminide ( $\text{TiAl}$ ) turbine blades, for example,  $\text{TiAl}$  low pressure turbine blades. The mold composition may provide the ability to cast near-net-shape parts that require less machining and/or treatment than parts made using conventional shell molds and gravity casting. As used herein, the expression “near-net-shape” implies that the initial production of an article is close to the final (net) shape of the article, reducing the need for further treatment, such as, extensive machining and surface finishing. As used herein, the term “turbine blade” refers to both steam turbine blades and gas turbine blades.

Accordingly, the present disclosure addresses the challenges of producing a mold, for example, an investment

mold, that does not react significantly with titanium and titanium aluminide alloys. In addition, according to some aspects of the disclosure, the strength and stability of the mold allow high pressure casting approaches, such as centrifugal casting. One of the technical advantages of this disclosure is that, in one aspect, the disclosure may improve the structural integrity of net shape casting that can be generated, for example, from calcium aluminate cement and alumina investment molds. The higher strength, for example, higher fatigue strength, allows lighter components to be fabricated. In addition, components having higher fatigue strength can last longer, and thus have lower life-cycle costs.

#### Casting Mold Composition

Aspects of the present disclosure provide a composition of matter for investment casting molds that can provide improved components of titanium and titanium alloys. In one aspect of the present disclosure, calcium monoaluminate can be provided in the form of calcium aluminate cement. Calcium aluminate cement may be referred to as a "cement" or "binder." In certain embodiments, calcium aluminate cement is mixed with alumina particulates to provide a castable investment mold mix. The calcium aluminate cement may be greater than about 30% by weight in the castable mold mix. In certain embodiments, the calcium aluminate cement is between about 30% and about 60% by weight in the castable mold mix. The use of greater than 30% by weight of calcium aluminate cement in the castable mold mix (casting mold composition) is a feature of the present disclosure. The selection of the appropriate calcium aluminate cement chemistry and alumina formulation are factors in the performance of the mold. In one aspect, a sufficient amount of calcium oxide may be provided in the mold composition in order to minimize reaction with the titanium alloy.

In one aspect, the mold composition, for example, the investment mold composition, may comprise a multi-phase mixture of calcium aluminate cement and alumina particles. The calcium aluminate cement may function as a binder, for example, the calcium aluminate cement binder may provide the main skeletal structure of the mold structure. The calcium aluminate cement may comprise a continuous phase in the mold and provide strength during curing, and casting. The mold composition may consist of calcium aluminate cement and alumina, that is, calcium aluminate cement and alumina may comprise substantially the only components of the mold composition, with little or no other components. In one embodiment, the present disclosure comprises a titanium-containing article casting-mold composition comprising calcium aluminate. In another embodiment, the casting-mold composition further comprises oxide particles, for example, hollow oxide particles. According to aspects of the disclosure, the oxide particles may be aluminum oxide particles, magnesium oxide particles, calcium oxide particles, zirconium oxide particles, titanium oxide particles, silicon oxide particles, combinations thereof, or compositions thereof. In one embodiment, the oxide particles may be a combination of one or more different oxide particles.

The casting-mold composition can further include aluminum oxide, for example, in the form of hollow particles, that is, particles having a hollow core or a substantially hollow core substantially surrounded by an oxide. These hollow aluminum oxide particles may comprise about 99% of aluminum oxide and have about 10 millimeter [mm] or less in outside dimension, such as, width or diameter. In one embodiment, the hollow aluminum oxide particles have about 1 millimeter [mm] or less in outside dimension, such

as, width or diameter. In another embodiment, the aluminum oxide comprises particles that may have outside dimensions that range from about 10 microns [ $\mu\text{m}$ ] to about 10,000 microns. In certain embodiments, the hollow oxide particles may comprise hollow alumina spheres (typically greater than 100 microns in diameter). The hollow alumina spheres may be incorporated into the casting-mold composition, and the hollow spheres may have a range of geometries, such as, round particles, or irregular aggregates. In certain embodiments, the alumina may include both round particles and hollow spheres. In one aspect, these geometries were found to increase the fluidity of the investment mold mixture. The enhanced fluidity may typically improve the surface finish and fidelity or accuracy of the surface features of the final casting produced from the mold.

The aluminum oxide comprises particles ranging in outside dimension from about 10 microns to about 10,000 microns. In certain embodiments, the aluminum oxide comprises particles that are less than about 500 microns in outside dimension, for example, diameter or width. The aluminum oxide may comprise from about 0.5% by weight to about 80% by weight of the casting-mold composition. Alternatively, the aluminum oxide comprises from about 40% by weight to about 60% by weight of the casting-mold composition. Alternatively, the aluminum oxide comprises from about 40% by weight to about 68% by weight of the casting-mold composition.

In one embodiment, the casting-mold composition further comprises calcium oxide. The calcium oxide may be greater than about 10% by weight and less than about 50% by weight of the casting-mold composition. The final mold typically may have a density of less than 2 grams/cubic centimeter and strength of greater than 500 pounds per square inch [psi]. In one embodiment, the calcium oxide is greater than about 30% by weight and less than about 50% by weight of the casting-mold composition. Alternatively, the calcium oxide is greater than about 25% by weight and less than about 35% by weight of the casting-mold composition.

One aspect of the present disclosure is a mold for casting a titanium-containing article, comprising: a calcium aluminate cement comprising calcium monoaluminate, calcium dialuminate, and mayenite, wherein the mold has an intrinsic facecoat of about 10 microns to about 250 microns between the bulk of the mold and the mold cavity. In one embodiment, the facecoat is a continuous intrinsic facecoat.

In a specific embodiment, the casting-mold composition of the present disclosure comprises a calcium aluminate cement. The calcium aluminate cement includes at least three phases or components comprising calcium and aluminum: calcium monoaluminate ( $\text{CaAl}_2\text{O}_4$ ), calcium dialuminate ( $\text{CaAl}_4\text{O}_7$ ), and mayenite ( $\text{Ca}_{12}\text{Al}_{14}\text{O}_{33}$ ). The weight fraction of calcium monoaluminate in the intrinsic facecoat may be more than 0.60 and the weight fraction of mayenite may be less than 0.10. In one embodiment, the calcium monoaluminate in the bulk of the mold comprises a weight fraction of about 0.05 to 0.95, and the calcium monoaluminate in the intrinsic facecoat is about 0.1 to 0.90. In another embodiment, the calcium dialuminate in the bulk of the mold comprises a weight fraction of about 0.05 to about 0.80, and the calcium dialuminate in the intrinsic facecoat is about 0.05 to 0.90. In yet another embodiment, the mayenite in the bulk of the mold composition comprises a weight fraction of about 0.01 to about 0.30, and the mayenite in the intrinsic facecoat is about 0.001 to 0.05.

The exact composition of the bulk of the mold and the intrinsic facecoat may differ. For example, the calcium

monoaluminate in the bulk of the mold comprises a weight fraction of about 0.05 to 0.95, and the calcium monoaluminate in the intrinsic facecoat is about 0.1 to 0.90; the calcium dialuminate in the bulk of the mold comprises a weight fraction of about 0.05 to about 0.80, and the calcium dialuminate in the intrinsic facecoat is about 0.05 to 0.90; and wherein the mayenite in the bulk of the mold composition comprises a weight fraction of about 0.01 to about 0.30, and the mayenite in the intrinsic facecoat is about 0.001 to 0.05.

The weight fraction of calcium monoaluminate in the calcium aluminate cement may be more than about 0.5, and the weight fraction of mayenite in the calcium aluminate cement may be less than about 0.15. In another embodiment, the calcium aluminate cement is more than 30% by weight of the casting-mold composition. In one embodiment, the calcium aluminate cement has a particle size of about 50 microns or less.

In one embodiment, the weight fractions of these phases that are suitable in the cement of the bulk of the mold are 0.05 to 0.95 of calcium monoaluminate, 0.05 to 0.80 of calcium dialuminate, and 0.01 to 0.30 of mayenite. In one embodiment, the weight fractions of these phases in the facecoat of the mold are 0.1-0.90 of calcium monoaluminate, 0.05-0.90 of calcium dialuminate, and 0.001-0.05 of mayenite. In another embodiment, the weight fraction of calcium monoaluminate in the facecoat is more than about 0.6, and the weight fraction of mayenite is less than about 0.1. In one embodiment, the weight fraction of calcium monoaluminate in the cement of the bulk of the mold is more than about 0.5, and weight fraction of mayenite is less than about 0.15.

In one embodiment, the calcium aluminate cement has a particle size of about 50 microns or less. A particle size of less than 50 microns is preferred for three reasons: first, the fine particle size is believed to promote the formation of hydraulic bonds during mold mixing and curing; second, the fine particle size is understood to promote inter-particle sintering during firing, and this can increase the mold strength; and third, the fine particle size is believed to improve the surface finish of the cast article produced in the mold. The calcium aluminate cement may be provided as powder, and can be used either in its intrinsic powder form, or in an agglomerated form, such as, as spray dried agglomerates. The calcium aluminate cement can also be pre-blended with fine-scale (for, example, less than 10 micron in size) alumina. The fine-scale alumina is believed to provide an increase in strength due to sintering during high-temperature firing. In certain instances, larger-scale alumina (that is, greater than 10 microns in size) may also be added with or without the fine-scale alumina.

The hollow alumina particles serve at least two functions: [1] they reduce the density and the weight of the mold, with minimal reduction in strength; strength levels of approximately 500 psi and above are obtained, with densities of approximately 2 g/cc and less; and [2] they reduce the elastic modulus of the mold and help to provide compliance during cool down of the mold and the component after casting. The increased compliance and crushability of the mold may reduce the tensile stresses on the component.

#### Calcium Aluminate Cement Composition

The calcium aluminate cement used in aspects of the disclosure typically comprises three phases or components of calcium and aluminum: calcium monoaluminate ( $\text{CaAl}_2\text{O}_4$ ), calcium dialuminate ( $\text{CaAl}_4\text{O}_7$ ), and mayenite ( $\text{Ca}_{12}\text{Al}_{14}\text{O}_{33}$ ). Calcium mono-aluminate is a hydraulic mineral present in calcium alumina cement. Calcium monoal-

minate's hydration contributes to the high early strength of the investment mold. Mayenite is desirable in the cement because it provides strength during the early stages of mold curing due to the fast formation of hydraulic bonds. The mayenite is, however, typically removed during heat treatment of the mold prior to casting.

In one aspect, the initial calcium aluminate cement formulation is typically not at thermodynamic equilibrium after firing in the cement manufacturing kiln. However, after 10 mold making and high-temperature firing, the mold composition moves towards a thermodynamically stable configuration, and this stability is advantageous for the subsequent casting process. In one embodiment, the weight fraction of calcium monoaluminate in the cement is greater than 0.5, and weight fraction of mayenite is less than 0.15. The mayenite is incorporated in the mold in both the bulk of the mold and the facecoat because it is a fast setting calcium aluminate and it is believed to provide the bulk of the mold and the facecoat with strength during the early stages of 15 curing. Curing may be performed at low temperatures, for example, temperatures between 15 degrees Celsius and 40 degrees Celsius because the fugitive wax pattern is temperature sensitive and loses its shape and properties on thermal exposure above about 35 degrees C. It is preferred to cure the mold at temperatures below 30 degrees C.

The calcium aluminate cement may typically be produced by mixing high purity alumina with high purity calcium oxide or calcium carbonate; the mixture of compounds is typically heated to a high temperature, for example, temperatures between 1000 and 1500 degrees C. in a furnace or kiln and allowed to react.

The resulting product, known in the art as cement "clinker," that is produced in the kiln is then crushed, ground, and sieved to produce a calcium aluminate cement of the preferred particle size. Further, the calcium aluminate cement is designed and processed to have a minimum quantity of impurities, such as, minimum amounts of silica, sodium and other alkali, and iron oxide. In one aspect, the target level for the calcium aluminate cement is that the sum of the  $\text{Na}_2\text{O}$ ,  $\text{SiO}_2$ ,  $\text{Fe}_2\text{O}_3$ , and  $\text{TiO}_2$  is less than about 2 weight percent. In one embodiment, the sum of the  $\text{Na}_2\text{O}$ ,  $\text{SiO}_2$ ,  $\text{Fe}_2\text{O}_3$ , and  $\text{TiO}_2$  is less than about 0.05 weight percent.

In one aspect of the disclosure, a calcium aluminate cement with bulk alumina concentrations over 35% weight 45 is alumina ( $\text{Al}_2\text{O}_3$ ) and less than 65% weight calcium oxide is provided. In a related embodiment, this weight of calcium oxide is less than 50%. In one example, the maximum alumina concentration of the cement may be about 88% (for example, about 12%  $\text{CaO}$ ). In one embodiment, the calcium aluminate cement is of high purity and contains up to 70% alumina. The weight fraction of calcium monoaluminate 50 may be maximized in the fired mold prior to casting. A minimum amount of calcium oxide may be required to minimize reaction between the casting alloy and the mold. If there is more than 50% calcium oxide in the cement, this can lead to phases such as mayenite and tricalcium aluminate, and these do not perform as well as the calcium monoaluminate during casting. The preferred range for calcium oxide is less than about 50% and greater than about 60 10% by weight.

As noted above, the three phases in the calcium aluminate cement/binder in the mold are calcium monoaluminate ( $\text{CaAl}_2\text{O}_4$ ), calcium dialuminate ( $\text{CaAl}_4\text{O}_7$ ), and mayenite ( $\text{Ca}_{12}\text{Al}_{14}\text{O}_{33}$ ). The calcium monoaluminate in the cement 65 that generates the facecoat has three advantages over other calcium aluminate phases: 1) The calcium monoaluminate is incorporated in the mold because it has a fast setting

## 11

response (although not as fast as mayenite) and it is believed to provide the mold with strength during the early stages of curing. The rapid generation of mold strength provides dimensional stability of the casting mold, and this feature improves the dimensional consistency of the final cast component. 2) The calcium monoaluminate is chemically stable with regard to the titanium and titanium aluminide alloys that are being cast. The calcium monoaluminate is preferred relative to the calcium dialuminate, and other calcium aluminate phases with higher alumina activity; these phases are more reactive with titanium and titanium aluminide alloys that are being cast. 3) The calcium monoaluminate and calcium dialuminate are low expansion phases and are understood to prevent the formation of high levels of stress in the mold during curing, dewaxing, and subsequent casting. The thermal expansion behavior of calcium monoaluminate is a close match with alumina.

## The Facecoat

In certain embodiments, the mold contains a continuous intrinsic facecoat between the bulk of mold and the mold cavity. The mold is designed to contain phases that provide improved mold strength during mold making, and the continuous facecoat is designed to provide increased resistance to reaction during casting. The molds are capable of casting at high pressure, which is desirable for net-shape casting methods. A casting mold composition, a facecoat composition, and preferred constituent phases for the facecoat and the bulk of the mold, have been identified that provide castings with improved properties.

The facecoat is defined as the region of the mold adjacent to the internal surface, or mold cavity in the mold. In one embodiment, the facecoat is generally considered to be a region about 100 microns thick. In order to be more effective, the facecoat is continuous. The region behind the facecoat and further away from the mold cavity is referred to as the bulk of the mold.

One aspect of the present disclosure is a facecoat composition of a mold that is used for casting a titanium-containing article, the facecoat composition comprising: calcium monoaluminate, calcium dialuminate, and mayenite, wherein the facecoat composition is an intrinsic facecoat, is about 10 microns to about 250 microns thick, and is located between the bulk of the mold and the surface of the mold that opens to the mold cavity. The facecoat comprises, in one example, of calcium aluminate with a particle size of less than about 50 microns.

The use of an intrinsic facecoat has advantages over the use of an extrinsic facecoat. Specifically, extrinsic facecoats in molds that are used for casting, such as yttria or zircon, can degenerate, crack, and spall during mold processing and casting, specifically higher pressure casting. The pieces of facecoat that become detached from the extrinsic facecoat can become entrained in the casting when the mold is filled with molten metal, and the ceramic facecoat becomes an inclusion in the final part. The inclusion reduces the mechanical performance of the component that is produced from the casting.

In one embodiment, the present disclosure provides an intrinsic facecoat composition for investment casting molds, and a bulk mold composition, that together can provide improved cast components of titanium and titanium alloys. In one embodiment, the mold comprises calcium aluminate cement and alumina particles. In one example, the calcium aluminate cement serves two functions. First the cement generates an in-situ facecoat in the cavity of the mold that is generated by removal of a fugitive pattern, and second it acts as a binder between the alumina particles in the bulk of the

## 12

5 mold behind the facecoat. In one embodiment, the bulk composition range for CaO in the mold is between 10 and 50 weight percent. In one embodiment, the composition of CaO in the facecoat is between 20 and 40 weight percent. In one embodiment, the final mold has a density of less than 2 grams/cubic centimeter and a strength of greater than 500 psi.

10 The mold may comprise the bulk of the mold and an intrinsic facecoat, with the bulk of the mold and the intrinsic facecoat having different compositions, and the intrinsic facecoat comprising calcium aluminate with a particle size of less than about 50 microns. The mold may comprise the bulk of the mold and an intrinsic facecoat, wherein the bulk of the mold and the intrinsic facecoat have different compositions and wherein the bulk of the mold comprises alumina particles larger than about 50 microns. The mold, in one example, comprises the bulk of the mold and an intrinsic facecoat, wherein the bulk of the mold comprises alumina particles larger than about 50 microns and the intrinsic facecoat comprises calcium aluminate particles less than about 50 microns in size.

20 Net shape casting approaches as provided for in the present disclosure allow parts that can be inspected with non destructive methods, such as x-ray, ultrasound, or eddy current, in greater detail and at lower costs. The difficulties associated with attenuation and scattering of the inspection radiation in oversized thick sections is reduced. Smaller defects can potentially be resolved, and this can provide 25 parts with improved mechanical performance.

30 The present disclosure provides a casting mold composition and a casting process that can provide improved components of titanium and titanium alloys. In one embodiment, the mold is constructed using calcium aluminate cement, or 35 binder, and alumina particles. In an embodiment, the mold contains an intrinsic facecoat between the bulk of mold and the mold cavity. The size of the particles in the facecoat are typically less than 50 microns. The size of the particles in the bulk of the mold can be larger than 50 microns. In one 40 embodiment, the size of the particles in the bulk of the mold are greater than 1 mm. In one embodiment, the size of the particles in the facecoat are less than 50 microns, and the size of the particles in the bulk of the mold are more than 50 microns. Generally, the facecoat is continuous intrinsic 45 facecoat, allowing it to be more effective.

50 The intrinsic facecoat may have, by weight fraction, at least 20 percent more calcium aluminate, at least 20 percent less alumina, and at least 50 percent less mayenite than does the bulk of the mold. The weight fraction of calcium monoaluminate in the intrinsic facecoat may have more than 0.60 and the weight fraction of mayenite may be less than 0.10. In one example, the calcium monoaluminate in the intrinsic facecoat comprises a weight fraction of 0.1 to 0.9; the calcium dialuminate in the intrinsic facecoat comprises a weight fraction of 0.05 to 0.90; and the mayenite in the intrinsic facecoat comprises a weight fraction of 0.001 to 0.05. The increased weight fraction of calcium monoaluminate in the intrinsic facecoat reduces the rate of reaction of the molten alloy with the mold during casting.

55 The intrinsic facecoat may have, by weight fraction, at least 20 percent more calcium monoaluminate than the bulk of the mold. The intrinsic facecoat may have, by weight fraction, at least 20 percent less alumina than the bulk of the mold. In one example, the intrinsic facecoat may have, by weight fraction, at least 20 percent more calcium aluminate, at least 20 percent less alumina, and at least 50 percent less mayenite than does the bulk of the mold.

In certain embodiments, the constituent phases of the facecoat, as well as the constituent phases of the bulk of the mold, are important to the properties of the casting. As disclosed herein, the facecoat of the mold provides minimum reaction with the alloy during casting, and as a result the mold provides castings with the required component properties. External properties of the casting include features such as shape, geometry, and surface finish. Internal properties of the casting include mechanical properties, microstructure, and defects (such as pores and inclusions) below a critical size.

With respect to constituent phases of the facecoat of the mold and the bulk of the mold, calcium monoaluminate ( $\text{CaAl}_2\text{O}_4$ ) is desirable for at least two reasons. First, calcium monoaluminate promotes hydraulic bond formation between the cement particles during the initial stages of mold making, and this hydraulic bonding provides mold strength during mold construction. Second, calcium monoaluminate experiences a very low rate of reaction with titanium and titanium aluminide based alloys.

In one embodiment, the facecoat comprises calcium monoaluminate ( $\text{CaAl}_2\text{O}_4$ ), calcium dialuminate ( $\text{CaAl}_4\text{O}_7$ ), and mayenite ( $\text{Ca}_{12}\text{Al}_{14}\text{O}_{33}$ ), and alumina. In one embodiment, the size of the particles in the facecoat are less than 50 microns. In the facecoat, the combination of calcium monoaluminate ( $\text{CaAl}_2\text{O}_4$ ), calcium dialuminate ( $\text{CaAl}_4\text{O}_7$ ) is more than 50 weight percent, and the alumina concentration is less than 50 weight percent. In one embodiment, there is more than 30 weight percent calcium monoaluminate ( $\text{CaAl}_2\text{O}_4$ ) in the facecoat. The region behind the facecoat and further away from the mold cavity is referred to as the bulk of the mold. In this bulk of the mold section, in one embodiment, the combination of calcium monoaluminate ( $\text{CaAl}_2\text{O}_4$ ), calcium dialuminate ( $\text{CaAl}_4\text{O}_7$ ) is less than 50 weight percent, and the alumina concentration in the bulk of the mold is greater than 50 weight percent.

Conventional investment mold compounds that consist of fused silica, cristobalite, gypsum, or the like, that are used in casting jewelry and dental prostheses are not suitable for casting reactive alloys, such as titanium alloys, because there is reaction between titanium and the investment mold. Any reaction between the molten alloy and the mold will deteriorate the properties of the final casting. The deterioration can be as simple as poor surface finish due to gas bubbles, or in more serious cases, the chemistry, microstructure, and properties of the casting can be compromised.

The challenge has been to produce an investment mold that does not react significantly with titanium and titanium aluminide alloys. In this regard, few if any prior poured ceramic investment compounds exist that meet the requirements for structural titanium and titanium aluminide alloys. There is a need for an investment mold that does not react significantly with titanium and titanium aluminide alloys. In prior approaches, in order to reduce the limitations of the conventional investment mold compounds, several additional mold materials were developed. For example, an investment compound was developed of an oxidation-expansion type in which magnesium oxide or zirconia was used as a main component and metallic zirconium was added to the main constituent to compensate for the shrinkage due to solidification of the cast metal.

However, prior art investment compounds have limitations. For example, the investment mold compound that is intended to compensate for the shrinkage due to the solidification of the cast metal by the oxidation-expansion of metallic zirconium is difficult to practice, for several reasons. First, a wax pattern is coated on its surface with the

new investment compound with zirconium and then the coated wax pattern is embedded in the conventional investment compound in an attempt to make the required amount of zirconium as small as possible; coating the wax with zirconium is very difficult and not highly repeatable. Second, waxes of complex shaped components can not be coated in a sufficiently uniform manner. In addition, the coated layer can come off the wax when the investment mold mix is placed externally around the coated layer and the pattern, with the result that titanium reacts with the externally placed investment mold mix.

The use of an intrinsic facecoat has significant advantages over the use of an extrinsic facecoat. Extrinsic facecoats that are used in casting titanium alloys are typically yttria based facecoats, or zirconia based facecoats. Specifically, extrinsic facecoats in molds that are used for casting can degenerate, crack, and spall during mold processing (such as removal of the fugitive pattern and firing) and casting. The pieces of facecoat that become detached from the extrinsic facecoat can become entrained in the casting when the mold is filled with molten metal, and the ceramic facecoat becomes an inclusion in the final part. The inclusion reduces the mechanical performance of the component that is produced from the casting.

The calcium aluminate cement is referred to as a cement or binder, and in one embodiment, it is mixed with alumina particulate to make a castable investment mold mix. The calcium aluminate cement is typically >30% by weight in the castable investment mold mix; the use of this proportion of calcium aluminate cement is a feature of the present disclosure because it favors formation of an intrinsic facecoat. Applicants found that the selection of the correct calcium aluminate cement chemistry and alumina formulation are important in determining the performance of the mold. In one example, in terms of the calcium aluminate cement, Applicants found that it is also necessary to have a particular amount of calcium oxide (CaO) in order to minimize reaction with the titanium alloy.

In one embodiment, the facecoat comprises of calcium aluminate cement with a particle size less than about 50 microns. In another embodiment, the particle size of the calcium aluminate cement is less than about 10 microns. In one example, the bulk of the mold has particles greater than 50 microns in size and can contain alumina.

The facecoat has less alumina and more calcium aluminate cement than the bulk of the mold. The intrinsic facecoat may have, by weight fraction, at least 20 percent more calcium aluminate, at least 20 percent less alumina, and at least 50 percent less mayenite than does the bulk of the mold. In one example, the calcium monoaluminate in the intrinsic facecoat comprises a weight fraction of 0.1 to 0.9; the calcium dialuminate in the intrinsic facecoat comprises a weight fraction of 0.05 to 0.90; and the mayenite in the intrinsic facecoat comprises a weight fraction of 0.001 to 0.05. The increased weight fraction of calcium monoaluminate and dialuminate in the intrinsic facecoat reduces the rate of reaction of the molten alloy with the mold during casting.

The initial cement slurry is mixed to have a viscosity of between 50 and 150 centipoise. In one embodiment, viscosity range is between 80 and 120 centipoise. If the viscosity is too low, the slurry will not maintain all the solids in suspension, and settling of the heavier particles will occur and lead to segregation during curing, and an intrinsic facecoat will not be formed. If the viscosity is too high, the calcium aluminate particles can not partition to the fugitive pattern, and the intrinsic facecoat will not be formed. The

final slurry with the calcium aluminate cement and the alumina particles is mixed to have a viscosity of between approximately 2000 and 8000 centipoise. In one embodiment, this final slurry viscosity range is between 3000 and 6000 centipoise. If the final slurry/mix viscosity is too high, the final slurry mix will not flow around the fugitive pattern, and the internal cavity of the mold will not be suitable for casting the final required part. If the final slurry mix viscosity is too low, settling of the heavier particles will occur during curing, and the mold will not have the required uniform composition throughout the bulk of the mold.

The investment mold consists of a multi-phase mixtures of fine-scale (<50 microns) calcium aluminate cement particles, fine-scale (<50 microns) alumina particles, and larger scale (>100 microns) alumina particles. The intrinsic facecoat does not contain any alumina particles greater than 50 microns. The intrinsic facecoat is formed because the fine-scale cement particles in suspension in the water-based investment mix partition preferentially to the fugitive/wax pattern during mold making, and forms an intrinsic facecoat layer that is enriched in the fine-scale particles (<50 microns), including the calcium monoaluminate, calcium dialuminate and alumina particles. In one embodiment, there are no large-scale alumina particles (>50 microns) in the facecoat. The slurry viscosity and the solids loading are factors in forming the intrinsic facecoat. The absence of large-scale (>100 micron) particles in the intrinsic facecoat improves the surface finish of the mold and the resulting casting. The increased weight fraction of calcium monoaluminate and dialuminate in the intrinsic facecoat reduces the rate of reaction of the molten alloy with the mold during casting.

In the bulk of the mold, the calcium aluminate cement is the binder, and the binder is considered the main skeleton of the mold structure behind the facecoat. It is the continuous phase in the mold and provides strength during curing, and casting. In one embodiment, the bulk of the mold composition comprises fine-scale (<50 microns) calcium aluminate cement particles, and larger scale (>100 microns) alumina particles. In another embodiment, the facecoat composition comprises calcium aluminate cement.

The calcium aluminate cement that makes up the facecoat comprises at least three phases; calcium monoaluminate ( $\text{CaAl}_2\text{O}_4$ ), calcium dialuminate ( $\text{CaAl}_4\text{O}_7$ ), and mayenite ( $\text{Ca}_{12}\text{Al}_{14}\text{O}_{33}$ ). In one embodiment, the facecoat can also contain fine-scale alumina particles. In another embodiment, the bulk of the mold behind the facecoat comprises calcium monoaluminate ( $\text{CaAl}_2\text{O}_4$ ), calcium dialuminate ( $\text{CaAl}_4\text{O}_7$ ), mayenite ( $\text{Ca}_{12}\text{Al}_{14}\text{O}_{33}$ ), and alumina. The alumina can be incorporated as alumina particles, for example hollow alumina particles. The particles can have a range of geometries, such as round particles, or irregular aggregates. The alumina particle size can be as small as 10 microns and as large as 10 mm.

In one embodiment, the alumina consists of both round particles and hollow particles, since these geometries increase the fluidity of the investment mold mixture. Typically the alumina particle size in the bulk of the mold is greater than 50 microns. The fluidity impacts the manner in which the cement partitions to the fugitive pattern (such as a wax) during pouring and setting of the investment mold mix around the fugitive pattern. The fluidity affects the surface finish and fidelity of the surface features of the final casting produced from the mold.

If the viscosity of the initial cement mix is too low, the slurry will not maintain all the solids in suspension, and settling of the heavier particles will occur and lead to

segregation during curing, and an intrinsic facecoat will not be formed. If the viscosity is too high, the calcium aluminate particles cannot partition to the fugitive pattern, and the intrinsic facecoat will not be formed. If the final mix viscosity is too high, the final slurry mix will not flow around the fugitive pattern, air will be trapped between the slurry mix and the pattern, and the internal cavity of the mold will not be suitable for casting the final required part. If the final slurry mix viscosity is too low, settling of the heavier particles will occur during curing, and the mold will not have the required uniform composition throughout the bulk of the mold, and the quality of the resulting casting will be compromised.

The calcium aluminate cement particulate that generates the facecoat typically has a particle size of less than 50 microns. A particle size of less than 50 microns has several advantages, including: first, the fine particle size promotes the formation of hydraulic bonds during mold mixing and curing, second the fine particle size can promote interparticle sintering during firing, and this can increase the mold strength, and third, the fine particle size improves surface finish of the mold cavity. The calcium aluminate cement powder can be used either in its intrinsic form, or in an agglomerated form, such as spray dried agglomerates. The calcium aluminate cement can also be preblended with fine-scale (<10 micron) alumina before mixing with larger-scale alumina; the fine-scale alumina can provide an increase in strength due to sintering during high-temperature firing. However, if the alumina particles partition to the facecoat, the casting properties can be reduced.

For example, if the alumina particles partition to the facecoat, such that the intrinsic facecoat has more alumina than the bulk of the mold, the molten alloy will react with the alumina in an undesirable way and generate gas bubbles that create surface defects and defects within the casting itself. The properties of the resulting casting, such as strength and fatigue strength are reduced. The presently disclosed methods allow for the formation of a facecoat that has significantly less alumina in the intrinsic facecoat than in the bulk of the mold.

The treatment of the facecoat and the mold from room temperature to the final firing temperature can also be important, specifically the thermal history and the humidity profile. The heating rate to the firing temperature, and the cooling rate after firing are very important. If the facecoat and the mold are heated too quickly, they can crack internally or externally, or both; facecoat and mold cracking prior to casting is highly undesirable, it will generate poor surface finish, at least. In addition, if the mold and facecoat are heated too quickly the facecoat of the mold can crack and spall off; this can lead to undesirable inclusions in the final casting in the worst case, and poor surface finish, even if there are no inclusions. If the facecoat and the mold are cooled too quickly after reaching the maximum mold firing temperature, the facecoat or the bulk of the mold can also crack internally or externally, or both.

The solids loading of the initial cement mix and the solids loading of the final mold mix have important effects on the mold structure and the ability to form an intrinsic facecoat within the mold, as will be described in the following paragraphs. The percentage of solids loading is defined as the total solids in the mix divided by the total mass of the liquid and solids in the mix, described as a percentage. In one embodiment, the percentage of solids in the initial calcium aluminate-liquid cement mix is about 71 percent to 78 percent.

If the solids loading in the initial cement slurry is less than about 70 percent, then the cement particles will not remain in suspension and during curing of the mold the cement particles will separate from the water and the composition will not be uniform throughout the mold. In contrast, if the solids loading is too high in the cement (for example greater than about 78 percent), the viscosity of the final mix with the large-scale alumina will be too high (for example greater than about 85%, depending on the amount, size, and morphology of the large-scale alumina particles that are added), and the cement particles in the mix will not be able to partition to the fugitive pattern within the mold, and the intrinsic facecoat will not be formed.

In one embodiment, the percentage of solids in the final calcium aluminate-liquid cement mix with the large-scale (meaning greater than about 50 microns in one embodiment, and greater than about 100 microns in another embodiment) alumina particles is about 75 percent to about 90 percent. In one embodiment, the percentage of solids in the final calcium aluminate-liquid cement mix with the large-scale alumina particles is about 78 percent to about 88 percent. In another embodiment, the percentage of solids in the final calcium aluminate-liquid cement mix with the large-scale alumina particles is about 78 percent to about 84 percent. In a particular embodiment, the percentage of solids in the final calcium aluminate-liquid cement mix with the large-scale alumina particles is about 80 percent.

#### The Mold and Casting Methods

An investment mold is formed by formulating the investment mix of the ceramic components, and pouring the mix into a vessel that contains a fugitive pattern. The investment mold formed on the pattern is allowed to cure thoroughly to form a so-called "green mold." The intrinsic facecoat and the investment mold are formed on the pattern and they are allowed to cure thoroughly to form this green mold. Typically, curing of the green mold is performed for times from 1 hour to 48 hours. Subsequently, the fugitive pattern is selectively removed from the green mold by melting, dissolution, ignition, or other known pattern removal technique. Typical methods for wax pattern removal include oven dewax (less than 150 degrees C.), furnace dewax (greater than 150 degrees C.), steam autoclave dewax, and microwave dewaxing.

For casting titanium alloys, and titanium aluminide and its alloys, the green mold then is fired at a temperature above 600 degrees C., for example 600 to 1400 degrees C., for a time period in excess of 1 hour, preferably 2 to 10 hours, to develop mold strength for casting and to remove any undesirable residual impurities in the mold, such as metallic species (Fe, Ni, Cr), and carbon-containing species. In one example, the firing temperature is at least 950 degrees C. The atmosphere of firing the mold is typically ambient air, although inert gas or a reducing gas atmosphere can be used.

The firing process also removes the water from the mold and converts the mayenite to calcium aluminate. Another purpose of the mold firing procedure is to minimize any free silica that remains in the facecoat and mold prior to casting. Other purposes are to increase the high temperature strength, and increase the amount of calcium monoaluminate and calcium dialuminate.

The mold is heated from room temperature to the final firing temperature, specifically the thermal history is controlled. The heating rate to the firing temperature, and the cooling rate after firing are typically regulated or controlled. If the mold is heated too quickly, it can crack internally or externally, or both; mold cracking prior to casting is highly undesirable. In addition, if the mold is heated too quickly,

the internal surface of the mold can crack and spall off. This can lead to undesirable inclusions in the final casting, and poor surface finish, even if there are no inclusions. Similarly, if the mold is cooled too quickly after reaching the maximum temperature, the mold can also crack internally or externally, or both.

The mold composition described in the present disclosure is particularly suitable for titanium and titanium aluminide alloys. The facecoat and the bulk of the mold composition 10 after firing and before casting can influence the mold properties, particularly with regard to the constituent phases. In one embodiment, for casting purposes, a high weight fraction of calcium monoaluminate in the mold is preferred, for example, a weight fraction of 0.15 to 0.8. In addition, for 15 casting purposes, it is desirable to minimize the weight fraction of the mayenite, for example, using a weight fraction of 0.01 to 0.2, because mayenite is water sensitive and it can provide problems with water release and gas 20 generation during casting. After firing, the mold can also contain small weight fractions of aluminosilicates and calcium aluminosilicates. The sum of the weight fraction of aluminosilicates and calcium aluminosilicates may typically be kept to less than 5% in the bulk of the mold and less than 0.5% in the facecoat, in order to minimize reaction of the 25 mold with the casting.

One aspect of the present disclosure is a method for forming a casting mold for casting a titanium-containing article, the method comprising: combining calcium aluminate with a liquid to produce a slurry of calcium aluminate, 30 wherein the percentage of solids in the initial calcium aluminate/liquid mixture is about 70% to about 80% and the viscosity of the slurry is about 50 to about 150 centipoise; adding oxide particles into the slurry such that the solids in the final calcium aluminate/liquid mixture with the large-scale (greater than 50 microns) oxide particles is about 75% to about 90%; introducing the slurry into a mold cavity that contains a fugitive pattern; and allowing the slurry to cure in the mold cavity to form a mold of a titanium-containing article.

40 In certain embodiments, the casting-mold composition of the present disclosure comprises an investment casting-mold composition. The investment casting-mold composition comprises a near-net-shape, titanium-containing metal, investment casting mold composition. In one embodiment, the investment casting-mold composition comprises an investment casting-mold composition for casting near-net-shape titanium aluminide articles. The near-net-shape titanium aluminide articles comprise, for example, near-net-shape titanium aluminide turbine blades.

45 The selection of the correct calcium aluminate cement chemistry and alumina formulation are factors in the performance of the mold during casting. In terms of the calcium aluminate cement, it may be necessary to minimize the amount of free calcium oxide in order to minimize reaction with the titanium alloy. If the calcium oxide concentration in the cement is less than about 10% by weight, the alloy reacts with the mold because the alumina concentration is too high, and the reaction generates undesirable oxygen concentration levels in the casting, gas bubbles, and a poor surface finish 50 in the cast component. Free alumina is less desirable in the mold material because it can react aggressively with titanium and titanium aluminide alloys.

55 If the calcium oxide concentration in the cement is greater than 50% by weight, the mold can be sensitive to pick up of water and carbon dioxide from the environment. As such, the calcium oxide concentration in the investment mold may 60 typically be kept below 50%. In one embodiment, the

calcium oxide concentration in the bulk of the investment mold is between 10% and 50% by weight. In one embodiment, the calcium oxide concentration in the bulk of the investment mold is between 10% and 40% by weight. Alternatively, the calcium oxide concentration in the bulk of the investment mold may be between 25% and 35% by weight. In one embodiment, the composition of CaO in the facecoat is between 20 and 40 percent by weight. In another embodiment, the calcium oxide concentration in the facecoat of the mold is between 15% and 30% by weight.

Carbon dioxide can lead to formation of calcium carbonate in the mold during processing and prior to casting, and calcium carbonate is unstable during the casting operation. Thus, the water and carbon dioxide in the mold can lead to poor casting quality. If the adsorbed water level is too high, for example, greater than 0.05 weight percent, when the molten metal enters the mold during casting, the water is released and it can react with the alloy. This leads to poor surface finish, gas bubbles in the casting, high oxygen concentration, and poor mechanical properties. In addition, an amount of water can cause the mold to be incompletely filled. Similarly, if the carbon dioxide level is too high, calcium carbonate can form in the mold and when the molten metal enters the mold during casting, the calcium carbonate can decompose generating carbon dioxide, which can react with the alloy; if large amounts of carbon dioxide are released, the gas can cause the mold to be incompletely filled. The resulting calcium carbonate is less than 1 weight percent in the mold.

Prior to casting a molten metal or alloy, the investment mold typically is preheated to a mold casting temperature that is dependent on the particular component geometry or alloy to be cast. For example, a typical mold preheat temperature is 600 degrees C. Typically, the mold temperature range is 450 degrees C. to 1200 degrees C.; the preferred temperature range is 450 degrees C. to 750 degrees C., and in certain cases it is 500 degrees C. to 650 degrees C.

According to one aspect, the molten metal or alloy is poured into the mold using conventional techniques which can include gravity, countergravity, pressure, centrifugal, and other casting techniques known to those skilled in the art. Vacuum or an inert gas atmospheres can be used. For complex shaped thin wall geometries, techniques that use high pressure are preferred. After the solidified titanium aluminide or alloy casting is cooled typically to less than 650 degrees, for example, to room temperature, it is removed from the mold and finished using conventional techniques, such as, grit blasting, and polishing.

One aspect of the present disclosure is a casting method for titanium and titanium alloys comprising: obtaining an investment casting mold composition comprising calcium aluminate and aluminum oxide, wherein the calcium aluminate is combined with a liquid to produce a slurry of calcium aluminate, and wherein the solids in the final calcium aluminate/liquid mixture with the large scale alumina is about 75% to about 90%, and wherein the resulting mold has an intrinsic facecoat; pouring the investment casting mold composition into a vessel containing a fugitive pattern; curing the investment casting mold composition; removing the fugitive pattern from the mold; firing the mold; preheating the mold to a mold casting temperature; pouring molten titanium or titanium alloy into the heated mold; solidifying the molten titanium or titanium alloy and forming a solidified titanium or titanium alloy casting; and removing the solidified titanium or titanium alloy casting from the mold.

In one embodiment, a titanium or titanium alloy article is claimed that is made by the casting method as taught herein.

One aspect of the present disclosure is directed to a casting method for titanium and titanium alloys comprising: 5 obtaining an investment casting-mold composition comprising calcium aluminate and aluminum oxide; pouring the investment casting-mold composition into a vessel containing a fugitive pattern; curing the investment casting-mold composition; removing the fugitive pattern from the mold; 10 firing the mold; preheating the mold to a mold casting temperature; pouring molten titanium or titanium alloy into the heated mold; solidifying the molten titanium or titanium alloy; and removing a solidified titanium or titanium alloy from the mold.

Between removing the fugitive pattern from the mold and preheating the mold to a mold casting temperature, the mold is first heated, or fired, to a temperature of about 600 degrees C. to about 1400 degrees C., for example about 950 degrees C. or higher, and then cooled to room temperature. In one embodiment, the curing step is conducted at temperatures below about 30 degrees C. for between one hour to 48 hours. The removing of the fugitive pattern includes the step of melting, dissolution, ignition, oven dewaxing, furnace dewaxing, steam autoclave dewaxing, or microwave dewaxing. In one embodiment, after removing of the titanium or titanium alloy from the mold, the casting may be finished with grit blasting or polishing. In one embodiment, after the solidified casting is removed from the mold, it is inspected 30 by X-ray or Neutron radiography.

The solidified casting is subjected to surface inspection and X-ray radiography after casting and finishing to detect any sub-surface inclusion particles at any location within the casting. X-ray radiography is employed to find inclusions 35 that are not detectable by visual inspection of the exterior surface of the casting. The titanium aluminide casting is subjected to X-ray radiography (film or digital) using conventional X-ray equipment to provide an X-ray radiograph that then is inspected or analyzed to determine if any sub-surface inclusions are present within the titanium aluminide casting.

Alternately or in addition to X-ray radiography, the solidified casting can be subjected to other non-destructive testing, for example, conventional Neutron-ray radiography. 45 The mold compositions described provide a small amount of a material having a high Neutron absorption cross section. In one aspect, a Neutron radiograph is prepared of the cast article. Since the titanium alloy cast article may be substantially transparent to neutrons, the mold material will typically show up distinctly in the resulting Neutron radiograph. In one aspect, it is believed that Neutron exposure results in “neutron activation” of the radiographically dense element. Neutron activation involves the interaction of the Neutron radiation with the radiographically dense element of the 55 casting to effect the formation of radioactive isotopes of the radiographically dense elements of the mold composition. The radioactive isotopes may then be detectable by conventional radioactive detecting devices to count any radiographically dense element isotopes present in the cast article.

Another aspect of the present disclosure is a method for forming a casting mold for casting a titanium-containing article. The method includes: combining calcium aluminate with a liquid, such as water, to produce a slurry of calcium aluminate in the liquid; introducing the slurry into a vessel 60 that contains a fugitive pattern; and allowing the slurry to cure in the mold cavity to form a mold of a titanium-containing article. In one embodiment, the method further

comprises, before introducing the slurry into a mold cavity, introducing oxide particles, for example hollow oxide particles, to the slurry.

The formed mold may be a green mold, and the method may further comprise firing the green mold. In one embodiment, the casting mold comprises an investment casting mold, for example, for casting a titanium-containing article. In one embodiment, the titanium-containing article comprises a titanium aluminide article. In one embodiment, the investment casting-mold composition comprises an investment casting-mold composition for casting near-net-shape titanium aluminide articles. The near-net-shape titanium aluminide articles may comprise near-net-shape titanium aluminide turbine blades. In one embodiment, the disclosure is directed to a mold formed from a titanium-containing article casting-mold composition, as taught herein. Another aspect of the present disclosure is directed to an article formed in the aforementioned mold.

Yet another aspect of the present disclosure is a titanium or titanium alloy casting made by a casting method comprising: obtaining an investment casting mold composition comprising calcium aluminate and aluminum oxide; pouring the investment casting mold composition into a vessel containing a fugitive pattern; curing the investment casting mold composition; removing the fugitive pattern from the mold; firing the mold; preheating the mold to a mold casting temperature; pouring molten titanium or titanium alloy into the heated mold; solidifying the molten titanium or titanium alloy to form the casting; and removing a solidified titanium or titanium alloy casting from the mold. In one embodiment, the present disclosure is directed to a titanium or titanium alloy article made by the casting methods taught in this application.

Surface roughness is one of the important indices representing the surface integrity of cast and machined parts. Surface roughness is characterized by the centerline average roughness value "Ra", as well as the average peak-to-valley distance "Rz" in a designated area as measured by optical profilometry. A roughness value can either be calculated on a profile or on a surface. The profile roughness parameter (Ra, Rq, . . .) are more common. Each of the roughness parameters is calculated using a formula for describing the surface. There are many different roughness parameters in use, but Ra is by far the most common. As known in the art, surface roughness is correlated with tool wear. Typically, the surface-finishing process though grinding and honing yields surfaces with Ra in a range of 0.1 mm to 1.6 mm. The surface roughness Ra value of the final coating depends upon the desired function of the coating or coated article.

The average roughness, Ra, is expressed in units of height. In the Imperial (English) system, 1 Ra is typically expressed in "millionths" of an inch. This is also referred to as "microinches". The Ra values indicated herein refer to microinches. An Ra value of 70 corresponds to approximately 2 microns; and an Ra value of 35 corresponds to approximately 1 micron. It is typically required that the surface of high performance articles, such as turbine blades, turbine vanes/nozzles, turbochargers, reciprocating engine valves, pistons, and the like, have an Ra of about 20 or less. One aspect of the present disclosure is a turbine blade comprising titanium or titanium alloy and having an average roughness, Ra, of less than 20 across at least a portion of its surface area.

As the molten metals are heated higher and higher, they tend to become more and more reactive (e.g., undergoing unwanted reactions with the mold surface). Such reactions lead to the formation of impurities that contaminate the

metal parts, which result in various detrimental consequences. The presence of impurities shifts the composition of the metal such that it may not meet the desired standard, thereby disallowing the use of the cast piece for the intended application. Moreover, the presence of the impurities can detrimentally affect the mechanical properties of the metallic material (e.g., lowering the strength of the material).

Furthermore, such reactions can lead to surface texturing, which results in substantial, undesirable roughness on the surface of the cast piece. For example, using the surface roughness value Ra, as known in the art for characterizing surface roughness, cast pieces utilizing stainless steel alloys and/or titanium alloys are typically exhibit an Ra value between about 100 and 200 under good working conditions. These detrimental effects drive one to use lower temperatures for filling molds. However, if the temperature of the molten metal is not heated enough, the casting material can cool too quickly, leading to incomplete filling of the cast mold.

One aspect of the present disclosure is directed to a mold composition for casting a titanium-containing article, comprising calcium aluminate. The mold composition further comprises hollow alumina particles. The article comprises a metallic article. In one embodiment, the article comprises a titanium aluminide-containing article. In another embodiment, the article comprises a titanium aluminide turbine blade. In yet another embodiment, the article comprises a near-net-shape, titanium aluminide turbine blade. This near-net-shape, titanium aluminide turbine blade may require little or no material removal prior to installation.

## EXAMPLES

The disclosure, having been generally described, may be more readily understood by reference to the following examples, which are included merely for purposes of illustration of certain aspects and embodiments of the present disclosure, and are not intended to limit the disclosure in any way.

FIGS. 1a and 1b show one example of the mold microstructure after high temperature firing. The backscattered electron scanning electron microscope images of the cross section of the mold fired at 1000 degrees Celsius are shown, wherein FIG. 1a points to the alumina particles 210 present, the mold facecoat 212, the bulk of the mold 214, and the internal surface of the mold 216 opening up to the mold cavity. FIG. 1b points to the calcium aluminate cement 220. The fine-scale calcium aluminate cement 220 provides the skeleton structure of the mold. In one example the calcium aluminate cement comprises calcium monoaluminate and calcium dialuminate.

FIG. 2a and FIG. 2b show one example of the mold microstructure after high temperature firing. The backscattered electron scanning electron microscope images of the cross section of the mold fired at 1000 degrees Celsius are shown, wherein FIG. 2a points to calcium aluminate cement 310 present as part of the facecoat microstructure. FIG. 2b points to an alumina particle 320 and shows the internal surface of mold/mold cavity 322 as well as the intrinsic facecoat region 324.

FIGS. 3 and 4 show two examples of the mold microstructure after high temperature firing, showing alumina 510 (in FIG. 3) 610 (in FIG. 4), and calcium monoaluminate 520 (in FIG. 3) 620 (in FIG. 4), wherein the mold in one example is fired to minimize mayenite content.

## Investment Mold Composition and Formulation

A calcium aluminate cement was mixed with alumina to generate an investment mold mix, and a range of investment mold chemistries were tested. The investment mixture in one example consisted of calcium aluminate cement with 70% alumina and 30% calcia, alumina particles, water, and colloidal silica.

As shown in FIG. 5a, the method 700 comprises combining calcium aluminate with a liquid to produce a slurry of calcium aluminate in the liquid 705. The percentage of solids in the initial calcium aluminate/liquid mixture is about 70% to about 80% and the viscosity of the slurry is about 50 to about 150 centipoise. In one embodiment oxide particles are added into the slurry 707 such that the solids in the final calcium aluminate/liquid mixture with the large scale (greater than 50 microns) oxide particles is about 75%-about 90%. The calcium aluminate slurry is introduced into a mold cavity that contains a fugitive pattern 710. The slurry is allowed to cure in the mold cavity to form a mold of a titanium or titanium-containing article 715.

In another example, shown in FIG. 5b, the method comprises obtaining an investment casting mold composition comprising calcium aluminate and aluminum oxide 725. In one example the calcium aluminate is combined with a liquid to produce a slurry of calcium aluminate, wherein the solids in the final calcium aluminate/liquid mixture with a large scale alumina is about 75% to about 90%. The investment casting mold composition is poured into a vessel containing a fugitive pattern 730. The investment casting mold is cured thereby providing the casting mold composition 735. The fugitive pattern is removed from the mold 740, and the mold is fired. The mold is preheated to a mold casting temperature 745, and the molten titanium or titanium alloy is poured into the heated mold 750. The molten titanium or titanium alloy is solidified and forms a solidified titanium or titanium alloy casting 755. Finally, the solidified titanium or titanium alloy casting is removed from the mold 760.

In a first example, a typical cement slurry mixture for making an investment mold consisted of 3000 grams [g] of the calcium aluminate cement, (comprising approximately 10% by weight of mayenite, approximately 70% by weight of calcium monoaluminate, and approximately 20% by weight of calcium dialuminate), 1500 g of calcined alumina particles with a size of less than 10 microns, 2450 g of high-purity alumina particles of a size range from 0.5 mm to 1.0 mm diameter, 1650 g of deionized water, and 150 g of colloidal silica. The solids loading of the final mold mix is 80 percent, where the solids loading is defined as the total solids in the mix normalized with respect to the total mass of the liquid and solids in the mix, expressed as a percentage.

The solids loading of the initial cement slurry mixture with all components and without the large-scale alumina particles is 72 percent. The mold formed an intrinsic facecoat with a thickness of approximately 100 microns. This formulation produced a mold that was approximately 120 mm diameter and 400 mm long. The mold formulation was designed so that there was less than 1 percent linear shrinkage of both the facecoat of the mold, and the bulk of the mold, on firing. The mold that was produced had a density of less than 2 grams per cubic centimeter.

Typical high-purity calcined alumina particles types include fused, tabular, and levigated alumina. Typical suitable colloidal silicas include REMASOL® LP30 (registered trademark of Remet PIC, Inc.), REMASOL® SP30, Nalco® 1030 (registered trademark of Ecolab USA Inc.), LUDOX® (registered trademark of W. R. GRACE & CO.). The pro-

duced mold was used for casting titanium aluminide-containing articles such as turbine blades with a good surface finish. The roughness (Ra) value was less than 100 micro-inches, and with an oxygen content of less than 2000 parts per million [ppm]. This formulation produced a mold that was approximately 120 mm diameter and 400 mm long. This formulation produced a mold that had a density of less than 2 grams per cubic centimeter.

The mold possessed an intrinsic facecoat that consisted of 10 calcium aluminate phases, and the facecoat thickness was approximately 100 microns. The mold that was so produced was used successfully for casting titanium aluminide turbine blades with a good surface finish; for example, where the Ra was less than 100, and with an oxygen content of less than 15 2000 ppm. This formulation produced a mold that had a density of less than 2 grams per cubic centimeter.

The mold mix was prepared by mixing the calcium aluminate cement, water, and colloidal silica in a container. A high-shear form mixing was used. If not mixed thoroughly, the cement can gel, and the fluidity is reduced so that the mold mix will not cover the fugitive pattern uniformly, and the intrinsic facecoat will not be generated. When the cement is in full suspension in the mixture, the alumina particles are added. When the cement was in full suspension 25 in the mixture, the fine-scale alumina particles were added. When the fine-scale alumina particles were fully mixed with the cement, the larger-size (for example, 0.5-1.0 mm) alumina particles were added and mixed with the cement-alumina formulation. The viscosity of the final mix is 30 another factor for the formation of a high quality facecoat continuous intrinsic facecoat, as it must not be too low or too high. Another key factor of the present disclosure is the solids loading of the cement mix and the amount of water. In addition, accelerants, and retarders can be used at selected 35 points during the mold making process steps.

After mixing, the investment mix was poured in a controlled manner into a vessel that contains the fugitive wax pattern. The vessel provides the external geometry of the mold, and the fugitive pattern generates the internal geometry. The correct pour speed is a further feature, if it is too fast air can be entrapped in the mold, if it is too slow separation of the cement and the alumina particulate can occur. Suitable pour speed range from about 1 to about 20 liters per minute. In one embodiment, the pour speed is about 2 to about 6 liters per minute. In a specific embodiment, the pour speed is about 4 liters per minute.

In a second example, a slurry mixture for making an investment mold consisted of 3000 g of the calcium aluminate cement, (comprising approximately 10% by weight of mayenite, approximately 70% by weight of calcium monoaluminate, and approximately 20% by weight of calcium dialuminate), 1500 g of calcined alumina particles with a size of less than 10 microns, 2650 g of high-purity alumina hollow particles of a size range from 0.5-1 mm diameter, 55 1650 g of deionized water, and 150 g of colloidal silica. After mixing, the investment mix was poured in a controlled manner into a vessel that contains the fugitive wax pattern, as described in the first example. The solids loading of the initial cement slurry mixture with all components without the large-scale alumina particles is 72 percent. The solids loading of the final mold mix is 80.3%; this is slightly higher 60 than the corresponding value in example one. The weight fraction of calcium aluminate cement is 42%, and that of the alumina is 58%. This formulation produced a mold that was approximately 120 mm diameter and 400 mm long.

The mold with the intrinsic facecoat was then cured and fired at high temperature. The mold with the intrinsic

facecoat that was so produced was used successfully for casting titanium aluminide turbine blades with a good surface finish; the Ra was less than 100, and with an oxygen content of less than 2000 ppm. This formulation produced a mold that had a density of less than 1.8 grams per cubic centimeter. The mold possessed an intrinsic facecoat comprising calcium aluminate phases. The mold formed an intrinsic facecoat with a thickness of approximately 100 microns. The mold formulation was designed so that there was less than 1 percent linear shrinkage of both the facecoat of the mold, and the bulk of the mold, on firing. The lightweight fused alumina hollow particles incorporated in the mix provides low thermal conductivity.

The alumina hollow particles provide a mold with a reduced density and lower thermal conductivity (the thermal conductivity is shown in the attached graph in FIG. 6). There is 35 weight percent of hollow alumina particles in the mold. This formulation produced a mold that was approximately 120 mm diameter and 400 mm long. The mold was then cured and fired at high temperature. The produced mold was used for casting titanium aluminide-containing articles, such as turbine blades, with a good surface finish. The roughness (Ra) value was less than 100, and with an oxygen content of less than 2000 ppm. This formulation produced a mold that had a density of less than 1.8 grams per cubic centimeter. The thermal conductivity of the bulk of the mold is compared with that of alumina in FIG. 6, as a function of temperature from room temperature to 1000° C. The thermal conductivity of the bulk of the mold is substantially less than that of alumina at all temperatures. The thermal conductivity was measured using hot wire platinum resistance thermometer technique (ASTM test C-1113).

In a third example, a slurry mixture for making an investment mold consisted of 600 g of the calcium aluminate cement, (consisting of approximately 10% by weight of mayenite, approximately 70% by weight of calcium monocaluminate, and approximately 20% by weight of calcium dialuminmate), 300 g of calcined alumina particles with a size of less than 10 microns, 490 g of high-purity alumina hollow particles of a size range from 0.5-1 mm diameter, 305 g of deionized water, and 31 g of REMASOL® LP30 colloidal silica. After mixing, the investment mix was poured in a controlled manner into a vessel that contains the fugitive wax pattern, as described in the first example. This formulation produced a smaller mold for a smaller component that was approximately 120 mm diameter and 150 mm long. The mold was then cured and fired at high temperature. The mold that was so produced was used successfully for casting titanium aluminide turbine blades with a good surface finish; the Ra was less than 100, and with an oxygen content of less than 1600 ppm.

The solids loading of the initial cement slurry mixture with all components without the large-scale alumina particles is 65 percent. This solids loading is below the ideal limit for making a cement slurry that can form a facecoat in the mold. The solids loading of the final mold mix is 77%; this is slightly lower than the preferred range for producing molds.

In a fourth example, a slurry mixture for making an investment mold consisted of 2708 g of a calcium aluminate cement, (comprising approximately 10% by weight of mayenite, approximately 70% by weight of calcium monocaluminate, and approximately 20% by weight of calcium dialuminmate), 1472 g of high-purity alumina hollow particles of a size range from 0.5-1 mm diameter, 1061 g of deionized water, and 96 g of REMASOL® colloidal silica LP30. After mixing, the investment mold mix was poured in a controlled

manner into a vessel that contains the fugitive wax pattern, as described in the first example. The solids loading of the initial cement slurry mixture with all components without the large-scale alumina particles is 70 percent. The solids loading of the final mold mix is 79%; this is slightly lower than the corresponding value in the first example. The mold formed an intrinsic facecoat with a thickness of approximately 100 microns. This formulation produced a smaller mold with a smaller alumina content for a smaller component. The mold was then cured and fired at high temperature. The produced mold was used for casting titanium aluminide-containing articles such as turbine blades.

In a fifth example, a slurry mixture for making an investment mold consisted of 1500 g of a commercially blended 80% calcium aluminate cement, CA25C, produced by the company ALAMATIS® (a registered trademark of ALMATIS, INC.). The CA25C product nominally consists of a 70% calcium aluminate cement blended with alumina to adjust the composition to 80% alumina. A cement slurry with an initial solids loading of 73.5 percent was produced using 460 g of deionized water, and 100 g of colloidal silica. When the slurry was mixed to an acceptable viscosity, 550 g of alumina hollow particles of a size range of less than 0.85 mm and greater than 0.5 mm was added to the slurry. The product with the name DURALUM® AB (a registered trademark of Washington Mills Company) that was produced by the company Washington Mills, was used. After mixing, the investment mold mix was poured in a controlled manner into a vessel that contains the fugitive wax pattern, as described in the first example. The solids loading of the final mold mix was 79.1%; this is on the low end of the preferred range. The mold mixture was poured into a tool to produce a mold with a diameter of 4 inches and a length of 6 inches.

The mold formed an intrinsic facecoat, but the composition of the bulk of the mold, and in particular the composition of the facecoat, contained too much silica. The bulk composition of silica in the mold was 1.4 weight percent. The high concentration of colloidal silica in the mix can lead to residual crystalline silica, and silicates, such as calcium aluminosilicate and aluminosilicate in the final fired mold. The high silica content of the mold, and the facecoat in particular, provided two limitations of this mold formulation. First, shrinkage can occur on firing and this leads to problems, such as cracking in the facecoat and dimensional control of the component. Second, the high silica content in the facecoat can cause reaction with the molten titanium and titanium aluminide alloys when the mold is filled during casting; this reaction leads to unacceptable casting quality.

In a sixth example, a mold with a diameter of 4 inches and a length of 6 inches was produced using a slurry mixture that consisted of 1500 g of a calcium aluminate cement, CA25C, 510 g of water, and 50 g of REMASOL® LP30 colloidal silica. This mix formulation possessed a lower colloidal silica concentration than the formulation in the previous example. The bulk composition of silica in the mold was 0.7 weight percent. The commercially blended 80% calcium aluminate cement, CA25C, was used. A cement slurry with an initial solids loading of 73.0 percent was produced. At this point, 550 g of DURALUM® AB alumina hollow particles of a size range of less than 0.85 mm and greater than 0.5 mm was added to the slurry. The solids loading of the final mold mix is 80.2%. After mixing, the investment mold mix was poured in a controlled manner into a vessel that contains the fugitive wax pattern, as described in the first example. The bulk composition of silica in the mold was 0.7 weight percent. The mold formed an intrinsic facecoat

with a lower silica content than that in the previous example. The lower silica content of the mold and in particular the intrinsic facecoat, provides a mold that is preferred for casting titanium and titanium aluminide alloys.

In a seventh example, a mold with a diameter of 100 millimeters and a length of 400 millimeters was produced using a slurry mixture that consisted of 4512 g of a calcium aluminate cement, CA25C, 1534 g of water, and 151 g of LP30 colloidal silica. A cement slurry with an initial solids loading of 73.0 percent was produced. The commercially blended 80% calcium aluminate cement, CA25C, was used. At this point, 2452 g of DURALUM® AB alumina hollow particles of a size range of less than 0.85 mm and greater than 0.5 mm, was added to the slurry. After mixing, the investment mold mix was poured in a controlled manner into a vessel that contains the fugitive wax pattern, as described in the first example. The solids loading of the final mold mix is 81%. The mold had a uniform composition along the 16 inch length of the mold in both the bulk of the mold, and the facecoat of the mold. The bulk composition of silica in the mold was 0.6 weight percent. The mold formed an intrinsic facecoat with a low silica content. The low silica content of the mold and in particular the intrinsic facecoat provides a mold that is preferred for casting titanium and titanium aluminide alloys. The weight percentage of alumina hollow particles in the mold was 35 percent. The mold formed an intrinsic facecoat with a thickness of approximately 100 microns. The mold experienced less than 1 percent linear shrinkage on firing.

In an eighth example, a mold with a diameter of 100 millimeters and a length of 150 millimeters was produced using a slurry mixture that consisted of 765 g of a commercially available calcium aluminate cement, Rescor 780, and REMASOL® LP30 colloidal silica. Rescor 780 is produced by Cotronics, Inc. The initial cement slurry mixed with the LP30 and possessed an initial solids loading of 76 percent. When the initial slurry had been mixed to a suitable viscosity, 1122 g of ZIRALCAST-95 was added. The solids loading of the final mold mix was 81%. After mixing, the investment mix was poured in a controlled manner into a vessel that contained the fugitive wax pattern, as described in the first example. The alumina castable refractory ZIRALCAST-95 is produced by ZIRCAR Ceramics, Inc. ZIRALCAST-95 is a high-purity alumina cement mixed with fused alumina hollow particles. The ZIRALCAST-95 contains approximately 44 percent alumina hollow particles by weight, and 56 percent alumina cement by weight; the alumina hollow particles size are larger than that used in the previous example, typically being greater than 1 mm.

This mold formulation that was so produced possessed some attractive attributes, but it possessed several limitations. First, the intrinsic facecoat in the mold was thinner than desired; this is due to high solids loading of the final mix prior to pouring. Second, there was too much colloidal silica in the mold mix and this led to too much silica, and resulting silicates, such as calcium aluminosilicate, in the bulk of the mold and in the facecoat of the final mold after firing. The high silica and silicate content of the mold and the facecoat in particular provided two limitations of this mold formulation. First, shrinkage can occur on firing and this leads to problems, such as cracking in the facecoat and dimensional control of the component. Second, the high silica content in the facecoat can cause reaction with the molten titanium aluminide alloy when the mold is filled during casting; this reaction leads to unacceptable casting quality. Lastly, the alumina hollow particles size was too large and this reduced the fluidity of the resulting mix. The

lower fluidity leads to a thinner intrinsic facecoat, and the resulting mold produces castings with lower quality.

In a ninth example, a slurry mixture was produced using 2708 g of a calcium aluminate cement, SECAR® 80 (a registered trademark of Kerneos Inc.), 820 g of deionized water, and 80 g of LP30 colloidal silica. SECAR® 80 cement is a commercially available hydraulic cement with an alumina content of approximately 80%. SECAR® 80 is produced by the company Kerneos, they were formerly known as LaFarge. The calcium aluminate cement clinker is prepared by solid-state reaction. The sintered clinker is then blended with high surface area alumina to create a hydraulic cement capable of contributing to high temperature strengths. The primary mineralogical phases of SECAR® 80 are calcium aluminate ( $\text{CaAl}_2\text{O}_4$ ), calcium di-aluminate ( $\text{CaAl}_4\text{O}_7$ ) and alumina ( $\text{Al}_2\text{O}_3$ ).

In a tenth example, a mold with a diameter of approximately 100 millimeters and a length of approximately 400 millimeters was produced using a slurry mixture that consisted of 4500 g of a calcium aluminate cement, CA25C and 1469 g of deionized water. A cement slurry with an initial solids loading of 75.3 percent was produced. The commercially blended 80% calcium aluminate cement, CA25C, was used. At this point, 2445 g of DURALUM® AB alumina hollow particles of a size range of less than 0.85 mm and greater than 0.5 mm, was added to the slurry. After mixing, the investment mold mix was poured in a controlled manner into a vessel that contains the fugitive wax pattern, as described in the first example. The solids loading of the final mold mix is 81%. The mold had a uniform composition along the 16 inch length of the mold in both the bulk of the mold, and the facecoat of the mold. The weight percentage of alumina hollow particles in the mold was 35 percent. The mold experienced less than 1 percent linear shrinkage on firing. The mold was suitable for casting.

A cement slurry with 2708 g of SECAR® 80 with an initial solids loading of 73.0 percent was produced. It was not possible to generate a slurry with this cement that could produce a mold with a preferred intrinsic facecoat. If the working time of the investment mold mix is too short, there is insufficient time to make large molds of complex-shaped components.

If the working time of the investment mold mix is too long and the calcium aluminate cement does not cure sufficiently quickly, separation of the fine-scale cement and the large scale alumina can occur and this can lead to a segregated mold in which the formulation varies and the resulting mold properties are not uniform.

The colloidal silica can affect the rate of reaction of the calcium aluminate phases with water, and it can also affect the mold strength during curing. This rate of reaction of the calcium aluminate phases with water controls the working time of the investment mold mix during mold making. This time was between about 30 seconds and about 10 minutes. If the working time of the investment mold mix is too short, there is insufficient time to make large molds of complex-shaped components, and the continuous intrinsic facecoat is not formed. If the working time of the investment mold mix is too long and the calcium aluminate cement does not cure sufficiently quickly, separation of the fine-scale cement and the large scale alumina can occur and this can lead to a segregated mold in which the formulation varies and the resulting mold properties are not uniform; it can also lead to the undesirable position of having a facecoat that is not continuous or varies in constituents and properties.

The constituent phases in the cement that makes up the continuous facecoat of the mold, and provides the binder for

the bulk of the mold, are a feature of the present disclosure. The three phases in the calcium aluminate cement comprises calcium monoaluminate ( $\text{CaAl}_2\text{O}_4$ ), calcium dialuminate ( $\text{CaAl}_4\text{O}_7$ ), and mayenite ( $\text{Ca}_{12}\text{Al}_{14}\text{O}_{33}$ ), and the inventors made this selection to achieve several purposes. First, the phases must dissolve or partially dissolve and form a suspension that can support all the aggregate phases in the subsequent investment mold making slurry. Second, the phases must promote setting or curing of the mold after pouring. Third, the phases must provide strength to the mold during and after casting. Fourth, the phases must exhibit minimum reaction with the titanium alloys that is cast in the mold. Fifth, the mold must have a suitable thermal expansion match with the titanium alloy casting in order to minimize the thermal stress on the part that is generated during post-solidification cooling.

The three phases in the calcium aluminate cement/binder in the mold and in the facecoat of the mold are calcium monoaluminate ( $\text{CaAl}_2\text{O}_4$ ), calcium dialuminate ( $\text{CaAl}_4\text{O}_7$ ), and mayenite ( $\text{Ca}_{12}\text{Al}_{14}\text{O}_{33}$ ). The mayenite is incorporated in the mold because it is a fast setting calcium aluminate and it provides the facecoat and the bulk of the mold with strength during the early stages of curing. Curing must be performed at low temperatures, because the fugitive wax pattern is temperature sensitive and loses its shape and properties on thermal exposure above  $\sim 35$  deg C. It is preferred to cure the mold at temperatures below 30 deg C.

It is to be understood that the above description is intended to be illustrative, and not restrictive. For example, the above-described embodiments (and/or aspects thereof) may be used in combination with each other. In addition, many modifications may be made to adapt a particular situation or material to the teachings of the various embodiments without departing from their scope. While the dimensions and types of materials described herein are intended to define the parameters of the various embodiments, they are by no means limiting and are merely exemplary. Many other embodiments will be apparent to those of skill in the art upon reviewing the above description. The scope of the various embodiments should, therefore, be determined with reference to the appended claims, along with the full scope of equivalents to which such claims are entitled. In the appended claims, the terms "including" and "in which" are used as the plain-English equivalents of the respective terms "comprising" and "wherein." Moreover, in the following claims, the terms "first," "second," and "third," etc. are used merely as labels, and are not intended to impose numerical requirements on their objects. Further, the limitations of the following claims are not written in means-plus-function format and are not intended to be interpreted based on 35 U.S.C. § 112, sixth paragraph, unless and until such claim limitations expressly use the phrase "means for" followed by a statement of function void of further structure. It is to be understood that not necessarily all such objects or advantages described above may be achieved in accordance with any particular embodiment. Thus, for example, those skilled in the art will recognize that the systems and techniques described herein may be embodied or carried out in a manner that achieves or optimizes one advantage or group of advantages as taught herein without necessarily achieving other objects or advantages as may be taught or suggested herein.

While the invention has been described in detail in connection with only a limited number of embodiments, it should be readily understood that the invention is not limited to such disclosed embodiments. Rather, the invention can be modified to incorporate any number of variations, altera-

tions, substitutions or equivalent arrangements not heretofore described, but which are commensurate with the spirit and scope of the invention. Additionally, while various embodiments of the invention have been described, it is to be understood that aspects of the disclosure may include only some of the described embodiments. Accordingly, the invention is not to be seen as limited by the foregoing description, but is only limited by the scope of the appended claims.

10 This written description uses examples to disclose the invention, including the best mode, and also to enable any person skilled in the art to practice the invention, including making and using any devices or systems and performing any incorporated methods. The patentable scope of the invention is defined by the claims, and may include other examples that occur to those skilled in the art. Such other examples are intended to be within the scope of the claims if they have structural elements that do not differ from the literal language of the claims, or if they include equivalent structural elements with insubstantial differences from the literal language of the claims.

The invention claimed is:

1. A method for forming a mold for casting a titanium-containing article, said method comprising:

combining calcium aluminate with a liquid to produce an initial slurry of calcium aluminate, wherein the percentage of solids in the initial slurry is about 70% to about 80% and a viscosity of the initial slurry is about 50 to about 150 centipoise;

adding oxide particles into the initial slurry to create a final slurry, wherein the percentage of solids in the final slurry is about 75% to about 90%;

introducing the final slurry into a mold cavity that contains a fugitive pattern; and

allowing the final slurry to cure in the mold cavity to form a mold of a titanium-containing article.

2. The method as recited in claim 1, wherein the percentage of solids in the initial slurry is about 71% to about 78%.

3. The method as recited in claim 1, wherein the percentage of solids in the final slurry is about 78% to about 88%.

4. The method as recited in claim 1, wherein a viscosity of the final slurry has a viscosity within a range of about 2,000 centipoise to about 8,000 centipoise.

5. The method as recited in claim 1, wherein the calcium aluminate comprises more than about 30% by weight of the final slurry.

6. The method as recited in claim 1, wherein the oxide particles are aluminum oxide particles.

7. The method as recited in claim 6, wherein the aluminum oxide particles are large scale aluminum oxide particles greater than 50 microns in size.

8. The method as recited in claim 7, further comprising adding fine scale aluminum oxide particles less than 50 microns in size to the calcium aluminate and the liquid to produce the initial slurry.

9. The method as recited in claim 8, wherein the large scale aluminum oxide particles are greater than 100 microns in size and the fine scale aluminum oxide particles are less than 10 microns in size.

10. The method as recited in claim 8, wherein the fine scale and large scale aluminum oxide particles collectively comprise from about 40% by weight to about 68% by weight of the final slurry.

11. The method as recited in claim 1, wherein the calcium aluminate comprises calcium monoaluminate, calcium dialuminate, and mayenite.

**31**

12. The method as recited in claim 1, wherein allowing the final slurry to cure in the mold cavity to form a mold of a titanium-containing article comprises allowing the final slurry to cure in the mold cavity to form a mold with an intrinsic facecoat.

13. A method for forming a mold for casting a titanium-containing article, said method comprising:

combining calcium aluminate with a liquid to produce an initial slurry of calcium aluminate, wherein the percentage of solids in the initial slurry is about 70% to about 80% and a viscosity of the initial slurry is about 50 to about 150 centipoise;

10 adding oxide particles into the initial slurry to create a final slurry, wherein the percentage of solids in the final slurry is about 75% to about 90% and a viscosity of the final slurry is about 2,000 to about 8,000 centipoise;

15 introducing the final slurry into a mold cavity that contains a fugitive pattern; and

allowing the final slurry to cure in the mold cavity to form a mold of a titanium-containing article.

**32**

14. The method as recited in claim 13, wherein a viscosity of the initial slurry is within a range of about 80 centipoise to about 120 centipoise.

15. The method as recited in claim 13, wherein a viscosity of the initial slurry is within a range of about 90 centipoise to about 110 centipoise.

16. The method as recited in claim 13, wherein the calcium aluminate comprises more than about 30% by weight of the final slurry.

10 17. The method as recited in claim 13, wherein the oxide particles are large scale aluminum oxide particles greater than 50 microns in size.

15 18. The method as recited in claim 17, further comprising adding fine scale aluminum oxide particles less than 50 microns in size to the calcium aluminate and the liquid to produce the initial slurry.

19. The method as recited in claim 18, wherein the large scale aluminum oxide particles are greater than 100 microns in size and the fine scale aluminum oxide particles are less than 10 microns in size.

\* \* \* \* \*